

## [54] NICKEL BASE ALLOYS OF IMPROVED PROPERTIES

[75] Inventor: Richard L. Kennedy, Monroe, N.C.

[73] Assignee: Teledyne, Inc., Los Angeles, Calif.

[22] Filed: Mar. 16, 1973

[21] Appl. No.: 342,074

## Related U.S. Application Data

[63] Continuation-in-part of Ser. No. 188,260, Oct. 12, 1971, abandoned.

[52] U.S. Cl. .... 75/122; 75/134 F; 75/170; 75/171

[51] Int. Cl. .... C22c 19/00

[58] Field of Search ..... 75/171, 170, 122, 134 F; 148/32, 32.5, 31

## [56]

## References Cited

## UNITED STATES PATENTS

|           |        |                    |        |
|-----------|--------|--------------------|--------|
| 3,399,058 | 8/1968 | Roush .....        | 75/171 |
| 3,575,734 | 4/1971 | Muzyka et al. .... | 75/171 |
| 3,754,902 | 8/1973 | Boone et al. ....  | 75/171 |

Primary Examiner—R. Dean

Attorney, Agent, or Firm—Richards, Shefte &amp; Pinckney

## [57]

## ABSTRACT

A yttrium addition, which may be made in the normal course of vacuum melting, is employed to improve high temperature properties and hot workability of nickel base alloys.

14 Claims, 2 Drawing Figures



Degree of cracking experienced on forging



*Fig. 1* Degree of cracking experienced on forging



*Fig. 2* Degree of edge cracking experienced on rolling

## NICKEL BASE ALLOYS OF IMPROVED PROPERTIES

### CROSS-REFERENCES TO RELATED APPLICATIONS

This application is a continuation-in-part of copending application Ser. No. 188,260, filed Oct. 12, 1971, and now abandoned.

### BACKGROUND OF THE INVENTION

It is generally well known by those familiar with the manufacture of nickel base alloys that the addition of extremely small quantities of certain elements can have pronounced effects on their properties. The elements boron and zirconium, for example, have been known for years to improve significantly the creep properties of many nickel base alloys, although these elements are not usually credited with improving workability.

Recently, magnesium has been recognized as improving both the elevated temperature properties and hot workability of this class of alloy (see U.S. Pat. No. 3,512,963 and No. 3,575,734). The addition of Mg to the nickel base alloys is quite difficult, however, since most of them are usually vacuum melted. Because of its low melting point and high vapor pressure at the melting temperature of these alloys, the amount of Mg retained in the cast product may be quite low in comparison to the amount added, frequently 50 per cent or less. The addition must therefore usually be made under a partial pressure of an inert gas to aid in retaining the highest possible percentage of the amount added. Even then, depending upon pressure, temperature, and time, the amount of Mg retained often varies to a degree which causes significant variations in workability and properties from heat to heat and between different ingots cast from the same master heat.

Further problems may occur due to the presence of a Mg addition in consumable vacuum arc remelting, which is the highly desirable second step of the double melting process in which an intermediate ingot cast in the first melting operation, commonly called an electrode, is consumably remelted under vacuum in a water-cooled copper crucible. Typically, additional Mg is lost in this operation. In order to retain a significant amount of Mg, it is again necessary to remelt under a partial pressure of an inert gas, such as argon or helium, which has a detrimental effect on ingot surface quality and resulting product yield.

A principal object of the present invention was to develop a method for improving the hot workability and elevated temperature properties of nickel base alloys,

and to obtain such alloys of improved nature in these respects. It was a further object to provide a process for accomplishing this result which is more compatible with the vacuum melting operations commonly employed on nickel base alloys.

It has been discovered that all of these objectives can be met by the addition of small amounts of yttrium (i.e., in the range from about 0.02 to about 0.15 weight per cent). Yttrium has been added as an alloying element to various high temperature alloys in the past (see, for example, U.S. Pat. No. 3,516,826, No. 3,346,378 and No. 3,202,506). The principal reason for its addition, however, has been to improve the resistance of the resulting alloy to corrosion at high temperature from O<sub>2</sub>, N<sub>2</sub>, S, V, Pb, etc. In general, the amount of yttrium usually added for this reason is considerably larger (up to 3 per cent) than that required or desirable in the present invention.

The beneficial effects of yttrium additions on hot workability and elevated temperature stress rupture properties have not been recognized before. The probable reason for this is that at the high concentrations heretofore used there is often a detrimental effect on both hot workability and elevated temperature mechanical properties.

### SUMMARY OF THE INVENTION

Basically, the method of the present invention involves vacuum melting a nickel base alloy in the usual manner. After the refining action of the vacuum treatment has been completed, the yttrium addition is made to the molten metal under vacuum conditions (i.e., less than  $50 \times 10^{-3}$  mm Hg). Yttrium may be added in pure (elemental) form or by means of a yttrium-bearing material, such as a master alloy (e.g., Y:Cr) or a commercial grade of yttrium in which certain rare earth metals remain admixed. The yttrium addition is delayed until late in the melt cycle because of its very great reactivity. This permits many of the contaminates with which yttrium might react to be removed prior to its addition, thus effectively reducing the amount required and also limiting the amount of time available for any adverse reaction between the melting crucible material and the yttrium. The advantages achieved according to the present invention by the addition of yttrium can also be obtained by introducing it in the course of air melting procedures for any nickel base alloys that are otherwise suited to air melting.

Nominal compositions of typical nickel base alloys which can be treated advantageously in accordance with this invention are given in Table I that follows.

TABLE I

| Alloy      | C   | Cr   | Mo | Co   | Ti   | Al  | Fe  | Ni    | Cb    | Other  |
|------------|-----|------|----|------|------|-----|-----|-------|-------|--------|
| 718        | .04 | 19.0 |    | 3.1  |      | 0.9 | 0.5 | 18.5  | Bal.* | 5.2    |
| X-750      | .04 | 15.5 |    |      |      | 2.5 | 0.8 | 6.8   | Bal.* | 1.0    |
| I-706      | .03 | 16.0 |    |      |      | 1.8 | 0.2 | Bal.* | 41.5  | 2.9    |
| 901        | .05 | 12.5 |    | 5.7  |      | 2.8 | 0.2 | Bal.* | 42.5  |        |
| 625        | .05 | 21.5 |    | 9.0  |      | 0.2 | 0.2 | 2.5   | Bal.* | 4.0    |
| IN-102     | .06 | 15.0 |    | 3.0  |      | .6  | .4  | 7.0   | Bal.* | 3.0    |
| INOR-8     | .06 | 7.0  |    | 16.8 |      |     |     | 2.5   | Bal.* |        |
| Hast X     | .10 | 22.0 |    | 9.0  | 1.5  |     |     | 18.5  | Bal.* | 0.6 W  |
| Hast B     | .03 |      |    | 28.0 |      |     |     | 5.5   | Bal.* | 0.4 V  |
| Hast C     | .04 | 15.5 |    | 16.0 |      |     |     | 5.5   | Bal.* | 3.8 W  |
| Hast W     | .06 | 5.0  |    | 24.5 |      |     |     | 5.5   | Bal.* | .30 V  |
| Illiium R  | .05 | 22.0 |    | 5.0  |      |     |     | 6.0   | Bal.* | 2.5 Cu |
| Illiium 98 | .04 | 28.0 |    | 8.3  |      |     |     | Bal.* |       | 5.3 Cu |
| Rene' 41   | .08 | 19.0 |    | 9.8  | 11.0 | 3.2 | 1.5 | Bal.* |       |        |

\*Bal = Balance essentially, including minor amounts of impurities and any or all of Mn, Si, B and Zr.

As illustrated by the foregoing tabulation, and as further reflected by the exemplary procedures and test data set forth below, the nickel base alloys subject to effective treatment according to the present invention are those in which cobalt, if present, does not exceed about 12 per cent, in which chromium, if present, does not exceed about 28 per cent, and in which titanium plus aluminum, if either or both is present, does not exceed about 5 per cent, all by weight. Beyond these limits it is not possible to predict the effect of a yttrium addition from data presently available, and as additions exceeding any of these limits materially is apt to introduce special conditions of uncertain effect, it is to nickel base alloys of the familiar sort falling within the foregoing limits and as illustrated by the foregoing tabulation that the present invention is directed.

The improvement obtained by the addition of yttrium varies with the type of alloy involved and with the amount of yttrium added. In the case of age-hardenable alloys the notable improvement is in high temperature or mechanical properties, as these alloys as a class hot work quite well if adequate temperature control is maintained. Those alloys that are not age-hardenable, however, have very poor hot workability as a class, and it is in this respect that significant improvement is obtained with such alloys.

As to the addition amount, the data that follow show effects through a yttrium addition range from about 0.02 to about 0.15 weight per cent, as mentioned earlier, and indicate disadvantage or at least lack of benefit above or below this range. The data further indicate a preferable range from about 0.05 to about 0.075 weight per cent yttrium.

#### DESCRIPTION OF THE DRAWINGS

4  
alloy with a composition of about 0.03% carbon, 18.8% chromium, 3.1% molybdenum, 0.9% titanium, 0.5% aluminum, 18.0% iron, 5.0% columbium, balance essentially nickel. Each of the heats was melted and refined in vacuum in the normal manner. The first electrode in the series (D871) was cast at a pressure of  $20 \times 10^{-3}$  mm Hg with no special additions. For the remaining heats (D872-7), the melt chamber was back-pressured with argon to about 80 mm Hg, following the refining cycle and just prior to casting, and an addition of yttrium (pure) or magnesium (as Mg:Ni master alloy) was made in the amount shown in Table II. All electrodes in this series were consumably arc remelted to 4 inch diameter ingots. The one formed from the 10 heat with no special additions (D871) was remelted in a vacuum of  $6 \times 10^{-3}$  mm Hg. The remaining electrodes were remelted under an argon partial pressure of 40 mm Hg in order to maintain a constant ingot surface condition. The pressure used on consumable remelting 15 is not considered to be a factor in mechanical properties, however, because of the small ingot size involved. The resulting ingots were rolled to  $\frac{3}{4}$  inch square bar using identical procedures in each case. The hot rolled bar was solution treated for 1 hour at 1,750°F., followed by air cooling and aging for 8 hours at 1,325°F., and then by furnace cooling at 100°F. per hour to 20 1,150°F., holding for an additional 8 hours, and air cooling. Upon completion of stress rupture testing at 1,200°F. and 110,000 psi, it was apparent as set forth in 25 Table II that the alloys treated with yttrium additions had rupture ductilities significantly in excess of those of the alloy with no additions. It was further observed that the yttrium treated alloys exhibited rupture ductilities 30 fully comparable to those of the magnesium treated alloys. 35

TABLE II

| Heat No. | Special Addition, Weight Percent | Rupture Life Hours | Elongation Percent | Reduction in Area Percent | Test Bar   |
|----------|----------------------------------|--------------------|--------------------|---------------------------|------------|
| D871     | None                             | 67.4<br>93.0       | 10.5<br>12.5       | 19.5<br>25.0              | CSN<br>CSN |
| D872     | 0.025 yttrium                    | 47.6               | 21.9               | 35.9                      | "          |
|          |                                  | 54.2               | 22.2               | 34.7                      | "          |
| D873     | 0.050 yttrium                    | 52.8               | 30.9               | 59.6                      | "          |
|          |                                  | 97.1               | 23.6               | 60.6                      | "          |
| D874     | 0.075 yttrium                    | 81.0               | 30.1               | 59.8                      | "          |
|          |                                  | 115.0              | 27.6               | 63.9                      | "          |
| D875     | 0.100 yttrium                    | 35.1               | 36.5               | 59.8                      | "          |
|          |                                  | 39.7               | 25.7               | 60.5                      | "          |
| D876     | 0.100 magnesium                  | 88.9               | 32.7               | 56.2                      | "          |
|          |                                  | 103.8              | 26.4               | 58.3                      | "          |
| D877     | 0.150 magnesium                  | 144.7              | 33.1               | 50.9                      | "          |
|          |                                  | 87.6               | 18.4               | 44.1                      | "          |

CSN = Combination smooth and notch test bar.

FIG. 1 consists of photographic illustrations of the degree of cracking experienced in forging with the various additions noted; and

55

FIG. 2 is a comparable illustration of the degree of edge cracking experienced in rolling.

#### DETAILED DESCRIPTION OF THE INVENTION

The following examples will serve to illustrate the significant effects that can be obtained by the addition of yttrium to nickel base alloys in accordance with the present invention.

#### EXAMPLE I

A series of 45-pound double vacuum melted ingots were prepared from a master melt of an age-hardenable

#### EXAMPLE II

It is well known in the industry that the alloy used in 60 Example I is subject to notch embrittlement under certain conditions of forging or heat treatment. To produce this effect, additional samples of the  $\frac{3}{4}$  inch square bar described in Example I were solution treated for 1 hour at 1,850°F., followed by water 65 quenching and aging as previously stated. Test samples were machined and tested in stress rupture at 1,200°F. and 110,000 psi with the results set forth in the following Table III.

TABLE III

| Heat No. | Special Addition, Weight Percent | Rupture Life Hours | Elongation Percent | RA Percent | Test Bar |
|----------|----------------------------------|--------------------|--------------------|------------|----------|
| D871     | None                             | 1.1                | N.B.*              |            | CSN      |
|          |                                  | 1.1                | N.B.*              |            | CSN      |
| D872     | 0.025 yttrium                    | 4.5                | N.B.*              |            | CSN      |
|          |                                  | 77.5               | 4.9                | 12.2       | CSN      |
| D873     | 0.050 yttrium                    | 158.9              | 7.3                | 13.1       | CSN      |
|          |                                  | 122.7              | 9.3                | 15.3       | CSN      |
| D874     | 0.075 yttrium                    | 79.9               | 5.1                | 10.0       | CSN      |
|          |                                  | 36.5               | 8.1                | 7.8        | CSN      |
| D876     | 0.100 magnesium                  | 93.4               | 7.7                | 13.2       | CSN      |
|          |                                  | 105.3              | 4.7"               | 9.9"       | CSN      |
| D877     | 0.150 magnesium                  | 103.2              | 3.9"               | 10.8"      | CSN      |
|          |                                  | 13.1               | 8.7"               | 7.8"       | CSN      |

\*N.B. = notch break

" = Broke outside of punch mark.

" = Broke within one diameter of punch mark.

CSN = Combination smooth and notch bar.

It is to be noted that the heat with no addition was severely notch embrittled by the foregoing heat treatment, failing in the notch after only 1.1 hours, while those heats containing yttrium additions resisted notch embrittlement and failed in the smooth section of the test bar in all cases but one.

## EXAMPLE III

A series of 12-pound ingots were prepared from a master melt of an alloy containing about 0.04% carbon, 21.0% chromium, 8.6% molybdenum, 0.10% aluminum, 2.5% iron, 3.7% columbium, balance essentially nickel. Each of the ingots was melted and refined in vacuum in the normal manner, with two ingots being cast sequentially from each of two 24-pound furnace charges. At the end of the normal refine cycle and just before pouring, an addition of 0.05 magnesium was made under an argon back pressure of 250 mm Hg to the molten metal in the first furnace charge. The first 12-pound ingot from this charge was then cast at this same pressure (D344-1). The furnace was evacuated again and the remaining molten metal of the charge was held for one hour under a vacuum of less than  $50 \times 10^{-3}$  mm Hg to effect complete removal of the initial magnesium added by means of vaporization. The second 12-pound ingot, considered to be magnesium free, was then cast (D344-2) at a pressure of  $15 \times 10^{-3}$  mm Hg. Yttrium additions were made to the second furnace charge and ingots cast sequentially to produce levels of 0.01% yttrium (D347-1) and 0.05% yttrium (D347-2). Pure yttrium was added at a vacuum level of  $12 \times 10^{-3}$  mm Hg and both ingots were cast at this same pressure.

All of the ingots were hot worked from nominal 2 inch square tapered ingot size to  $\frac{3}{8} \times 1 \frac{1}{2}$  inch flat bar by forging and rolling. The same procedures were used on each. Hot workability of the heat to which 0.05% yttrium had been added (D347-2) was very good and essentially the same as that of the heat to which 0.05 Mg had been added (D344-1). Workability of the heat with a 0.01% yttrium addition (D347-1) was poor but was significantly better than the heat to which magnesium had been added and then removed by holding under vacuum (D344-2). These results can be seen from FIGS. I and II and Table IV.

TABLE IV

| Heat No. | Special Addition, Percent | Hot Workability |
|----------|---------------------------|-----------------|
| D344-1   | 0.05% magnesium           | Good            |
| D344-2   | —                         | Very Poor       |
| D347-1   | 0.01% yttrium             | Poor            |

TABLE IV-continued

| Heat No. | Special Addition, Percent | Hot Workability |
|----------|---------------------------|-----------------|
| D347-2   | 0.05% yttrium             | Good            |

Elevated temperature tensile testing was conducted as another measure of hot workability on bars cut from the heat having the 0.05% yttrium addition (D347-2). Reduction in area is generally regarded as an indication of hot workability according to this test. The results on this heat confirmed the good workability observed in rolling with values of 90 to 99% reduction in area over the temperature range of 2,200° to 1,700°F. At 2,150°F. the reduction in area of 92.4% compared very favorably with the result from the heat with the 0.05% magnesium addition which was 88.5%. Previous tests on other heats of this alloy with proven poor workability had a maximum value over this same temperature range of 60% reduction in area.

As an additional check on this experiment, a 45-pound heat of essentially this same composition (Heat No. D407) was melted from virgin raw materials. After vacuum refining in the normal manner and adding the usual late additions, 0.05% yttrium was added under a vacuum of  $12 \times 10^{-3}$  mm of Hg and the heat was poured. The resulting electrode was vacuum arc remelted at  $3 \times 10^{-3}$  mm of Hg to produce a 4 inch diameter ingot which was subsequently rolled to 0.440 inch diameter bar. Workability was rated as good based on actual mill observation, and by virtue of the fact that the small diameter bar was rolled essentially crack free. Elevated temperature tensile tests resulted in values of reduction in area ranging from 99.0% at 1,700°F. to 72.3% at 2,100°F. Although slightly lower than results on the 12-pound ingots, these values are still significantly above the 60% reduction in area maximum values experienced on the heats with extremely poor hot workability.

## EXAMPLE IV

Two 25-pound ingots of nominal 3 inch square tapered size were prepared from virgin raw materials with compositions of about 0.06% carbon, 15.4% chromium, 6.9% iron, 2.8% titanium, 0.85% aluminum, 1.1% columbium, balance essentially nickel. Both heats were melted and refined in vacuum in the normal manner. The first heat (G049) was cast with no special additions at a vacuum of  $23 \times 10^{-3}$  mm Hg. To the second heat in the series (G052), 0.05% yttrium was added

under a vacuum of  $20 \times 10^{-3}$  mm Hg and the ingot cast at this same pressure. Both ingots were forged to 1-1/4 inch square bar using identical hot working procedures. Bar samples from each heat were solution heat treated for 2 hours at 2,100°F., followed by air cooling and aging for 24 hours at 1,550°F. and 20 hours at 1,300°F. followed by air cooling. Stress rupture testing performed on these heat treated samples gave the results shown in Table V.

TABLE V

| Heat No. | Special Addition, Weight Percent | Test Temp. (°F.) | Stress ksi           | Rupture Life Hrs.        | Elongation Percent | Reduction in Area Percent |
|----------|----------------------------------|------------------|----------------------|--------------------------|--------------------|---------------------------|
| G049     | None                             | 1350             | 45/55 <sup>(1)</sup> | 703/750.5 <sup>(1)</sup> | 3.2                | 7.7                       |
|          |                                  | 1350             | 45/55 <sup>(1)</sup> | 703/734.9 <sup>(1)</sup> | 3.5                | 9.3                       |
|          |                                  | 1350             | 60                   | 158.0                    | 7.9                | 7.7                       |
| G052     | 0.050 yttrium                    | 1350             | 45/55 <sup>(1)</sup> | 703/863.7 <sup>(1)</sup> | 6.9                | 21.6                      |
|          |                                  | 1350             | 45/55 <sup>(1)</sup> | 703/747.5 <sup>(1)</sup> | 8.1                | 22.3                      |
|          |                                  | 1350             | 60                   | 241.0                    | 13.6               | 22.4                      |

<sup>(1)</sup>Stress increased from 45 to 55 ksi at 703 hours on each bar.

It is apparent from these data that the addition of yttrium resulted in approximately a doubling of rupture ductility for any given life, and at the same time produced some increase in rupture life under conditions of identical stress.

## EXAMPLE V

A group of solution hardened alloys were prepared with compositions as shown in Table VI below.

TABLE VI

| Heat No. | Y added (% by Wt.) | C   | Cr   | Mo   | Co  | Fe   | Ni    | Other      |
|----------|--------------------|-----|------|------|-----|------|-------|------------|
| D422     | .05                | .01 | 5.8  | 24.1 | .7  | 5.7  | Bal.* | .12V       |
| D432     | .05                | .10 | 21.4 | 8.9  | 2.3 | 19.0 | Bal.* |            |
| D454     | .05                | .03 | 0.3  | 26.3 | .2  | 5.5  | Bal.* | .3V        |
| D455     | .05                | .05 | 13.0 | 17.1 | —   | 6.8  | Bal.* | .15V, 3.4W |

\*Balance essentially, including minor amounts of impurities and any or all of Mn, Si, B, Zr.

Based on actual production experience, it is well known that the hot workability of all of these alloys is very poor unless they contain some special addition such as magnesium. Each of these alloys was melted and refined in vacuum in the usual manner. Yttrium additions of 0.05% were made to the molten charge shortly before casting in each case at vacuum levels of  $3 \text{ to } 12 \times 10^{-3}$  mm Hg. Electrodes from Heats D422, D454 and D455 were then vacuum arc remelted to 4 inch diameter ingots at vacuum levels of  $2 \text{ to } 8 \times 10^{-3}$  mm Hg. Heat D432 was prepared as a 4 inch square static cast ingot from the initial vacuum induction melt, and remelting was not performed on it. Each of these ingots was hot worked by rolling in a manner typical for that alloy. An initial breakdown operation was performed after which light grinding was required on each ingot except D432 to remove minor defects typical of those resulting from the as-cast ingot surface. No conditioning was required on the static cast ingot (Heat D432). Following this operation, bar product was rolled from each heat with no evidence of cracking. Hot workability was judged excellent in all cases.

Elevated temperature tensile testing was performed on bar rolled from Heat D455 over the temperature range of 1,700° to 2,200°F. Reduction in area, considered to be a rough measure of hot workability, ranged from 96.4 to 98.4% over this entire temperature spread, correlating very well with the favorable bar

rolling experience. Similar data collected on a good working heat with a magnesium addition ranged from 97.8 to 81.2%, while data from a heat with extremely poor workability showed a maximum value of 20% reduction in area. From these data it is apparent that the addition of yttrium produced a significant improvement in the hot workability of this group of alloys.

## EXAMPLE VI

A series of 47-pound double vacuum melted heats were made of an age-hardening alloy with a composition of about 0.03% carbon, 15.2% chromium, 41.5% nickel, 2.8% columbium, 1.6% titanium, 0.25% aluminum, 0.005% boron and balance essentially iron. Each heat was prepared from a master melt of this same alloy in order to keep the base chemistry as consistent as possible. All the heats were vacuum melted and refined in the normal manner with the exception of Heat G081

to which a special sulfur reducing slag was added. Yttrium additions were made under full vacuum just prior to pouring to selected heats as shown in Table VII. A magnesium addition was made to Heat G169, also just prior to pouring, but under a partial pressure of argon gas. Commercially available forms of yttrium of 95 and 99 per cent purities were employed. The magnesium addition was made as a Ni-Mg master alloy. All electrodes were vacuum arc remelted into 4 inch diameter ingots. The control heats, those to which no additions had been made, and the yttrium containing heats were remelted under full vacuum, although the pressure varied slightly as shown in Table VII. The magnesium containing heat was remelted under an argon partial pressure of 150 mm Hg. All other melting conditions were identical.

Since the alloy employed in this experiment is used in some cases as a casting alloy, testing was performed on samples sectioned directly from the as-cast ingots. Test bars were machined from the same position from each of the ingots prepared. These samples were heat treated by heating to 2,000°F. for 1 hour followed by air cooling, reheated to 1,800°F. for 1 hour, air cooled, reheated to 1,550°F. for 3 hours, air cooled, reheated to 1,325°F. for 8 hours followed by furnace cooling to 1,150°F. and holding until a total aging time of 18 hours had accumulated. Samples from each of the heats were tested in stress rupture at 1,200°F., and

90,000 psi. The results of this testing, as summarized in Table VIII, show a significant improvement in stress rupture ductility for heats with yttrium additions of 0.05 and 0.15% (G093, G094, G155) over all other heats prepared. In one case, on Heat G155, a slightly low stress rupture ductility of 6.2% elongation was encountered. This value is still greater than that of any obtained on control heats (no yttrium additions) or the magnesium containing heat, in spite of the fact that the test failure was within one diameter of the punch which almost always significantly reduces ductility.

There are also significant variations in rupture life illustrated by the data in Table VIII. Heats G093 and G155 containing 0.05 per cent yttrium additions displayed the highest average rupture lives of any of the other heats studied. The heat with a 0.15 per cent yttrium addition (G094) had a lower rupture life, on the average, than either the control heat (G081) or the 0.02 per cent yttrium containing heat (G083) but approximately equivalent to the magnesium bearing heat (G169).

TABLE VII

| Heat No. | Addition, Amount - Purity | Pressure at Time of Add mm | Pressure at Pour mm | VAR Pressure mm |
|----------|---------------------------|----------------------------|---------------------|-----------------|
| G080     | None                      |                            | .023                | .013            |
| G081     | None                      |                            | .030                | .015            |
| G083     | .02 yttrium - 99%         | .018                       | .018                | .013            |
| G093     | .05 yttrium - 99%         | .021                       | .020                | .002            |
| G094     | .15 yttrium - 99%         | .022                       | .025                | .003            |
| G153     | None                      |                            | .013                | .005            |
| G155     | .05 yttrium - 95%         | .011                       | .011                | .005            |
| G169     | .05 magnesium - 5%        | 75.0                       | 75.0                | 150.0           |

TABLE VIII

| Heat No. | Addition, Weight Percent | Rupture Life Hrs. | % El | % RA  |
|----------|--------------------------|-------------------|------|-------|
| G080     | None                     | 57.5              | 4.6  | 10.8  |
|          |                          | 38.5              | 4.5  | 5.5   |
| G081     | None                     | 317.9             | 4.8  | 4.7   |
|          |                          | 174.3             | 4.4  | 8.7   |
| G083     | .02 yttrium              | 138.8             | 6.9  | 6.3   |
|          |                          | 314.1             | 4.3  | 6.9   |
| G093     | .05 yttrium              | 401.1             | 8.7  | 12.9  |
|          |                          | 326.5             | 10.4 | 30.6  |
| G094     | .15 yttrium              | 104.4             | 9.5  | 19.0  |
|          |                          | 118.9             | 9.9  | 23.2  |
| G153     | None                     | 24.8              | 3.5  | 12.3  |
|          |                          | 26.0              | 4.6  | 8.6   |
| G155     | .05 yttrium              | 319.8             | 6.2  | 11.6* |
|          |                          | 220.4             | 15.6 | 29.8  |
| G169     | .05 magnesium            | 116.4             | 3.5  | 10.9  |

\*Broke within one diameter of punch mark.

The present invention has been described in detail above for purposes of illustration only and is not intended to be limited by this description or otherwise to exclude any variation or equivalent form or procedure that would be apparent from, or reasonably suggested by, the foregoing disclosure to the skill of the art.

I claim:

1. A nickel base alloy of improved characteristics in at least one of stress rupture properties and hot workability, said alloy having a nominal composition consisting essentially of about 0.04% carbon, about 19% chromium, about 3.1% molybdenum, about 0.9% titanium, about 0.5% aluminum, about 18.5% iron, about 5.2% columbium, and a balance that is essentially nickel except for an addition in said alloy of yttrium in an amount ranging from about 0.02% to about 0.15%.

2. A nickel base alloy of improved characteristics in at least one of stress rupture properties and hot workability, said alloy having a nominal composition consisting essentially of about 0.04% carbon, about 15.5% chromium, about 2.5% titanium, about 0.8% aluminum, about 6.8% iron, about 1.0% columbium, and a balance that is essentially nickel except for an addition in said alloy of yttrium in an amount ranging from about 0.02% to about 0.15%.

10 3. A nickel base alloy of improved characteristics in at least one of stress rupture properties and hot workability, said alloy having a nominal composition consisting essentially of about 0.03% carbon, about 16% chromium, about 1.8% titanium, about 0.2% aluminum, about 41.5% nickel, about 2.9% columbium, and a balance that is essentially iron except for an addition in said alloy of yttrium in an amount ranging from about 0.02% to about 0.15%.

15 4. A nickel base alloy of improved characteristics in at least one of stress rupture properties and hot workability, said alloy having a nominal composition consisting essentially of about 0.05% carbon, about 12.5% chromium, about 5.7% molybdenum, about 2.8% titanium, about 0.2% aluminum, about 42.5% nickel, and a balance that is essentially iron except for an addition in said alloy of yttrium in an amount ranging from about 0.02% to about 0.15%.

20 5. A nickel base alloy of improved characteristics in at least one of stress rupture properties and hot workability, said alloy having a nominal composition consisting essentially of about 0.05% carbon, about 21.5% chromium, about 9.0% molybdenum, about 0.2% titanium, about 0.2% aluminum, about 2.5% iron, about 4.0% columbium, and a balance that is essentially nickel except for an addition in said alloy of yttrium in an amount ranging from about 0.02% to about 0.15%.

25 6. A nickel base alloy of improved characteristics in at least one of stress rupture properties and hot workability, said alloy having a nominal composition consisting essentially of about 0.06% carbon, about 15% chromium, about 3.0% molybdenum, about 0.6% titanium, about 0.4% aluminum, about 7.0% iron, about 3.0% columbium, about 3.0% tungsten, and a balance that is essentially nickel except for an addition in said alloy of yttrium in an amount ranging from about 0.02% to about 0.15%.

30 7. A nickel base alloy of improved characteristics in at least one of stress rupture properties and hot workability, said alloy having a nominal composition consisting essentially of about 0.06% carbon, about 7.0% chromium, about 16.8% molybdenum, about 2.5% iron, and a balance that is essentially nickel except for an addition in said alloy of yttrium in an amount ranging from about 0.02% to about 0.15%.

35 8. A nickel base alloy of improved characteristics in at least one of stress rupture properties and hot workability, said alloy having a nominal composition consisting essentially of about 0.10% carbon, about 22% chromium, about 9.0% molybdenum, about 1.5% cobalt, about 18.5% iron, about 0.6% tungsten, and a balance that is essentially nickel except for an addition in said alloy of yttrium in an amount ranging from about 0.02% to about 0.15%.

40 9. A nickel base alloy of improved characteristics in at least one of stress rupture properties and hot workability, said alloy having a nominal composition consisting essentially of about 0.03% carbon, about 28% molybdenum, about 5.5% iron, about 0.4% vanadium,

and a balance that is essentially nickel except for an addition in said alloy of yttrium in an amount ranging from about 0.02% to about 0.15%.

10. A nickel base alloy of improved characteristics in at least one of stress rupture properties and hot workability, said alloy having a nominal composition consisting essentially of about 0.04% carbon, about 15.5% chromium, about 16% molybdenum, about 5.5% iron, about 3.8% tungsten, and a balance that is essentially nickel except for an addition in said alloy of yttrium in an amount ranging from about 0.02% to about 0.15%.

11. A nickel base alloy of improved characteristics in at least one of stress rupture properties and hot workability, said alloy having a nominal composition consisting essentially of about 0.06% carbon, about 5.0% chromium, about 24.5% molybdenum, about 5.5% iron, about 0.3% vanadium, and a balance that is essentially nickel except for an addition in said alloy of yttrium in an amount ranging from about 0.02% to about 0.15%.

12. A nickel base alloy of improved characteristics in at least one of stress rupture properties and hot workability, said alloy having a nominal composition con-

sisting essentially of about 0.05% carbon, about 22% chromium, about 5.0% molybdenum, about 6.0% iron, about 2.5% copper, and a balance that is essentially nickel except for an addition in said alloy of yttrium in an amount ranging from about 0.02% to about 0.15%.

13. A nickel base alloy of improved characteristics in at least one of stress rupture properties and hot workability, said alloy having a nominal composition consisting essentially of about 0.04% carbon, about 28% chromium, about 8.3% molybdenum, about 5.3% copper, and a balance that is essentially nickel except for an addition in said alloy of yttrium in an amount ranging from about 0.02% to about 0.15%.

14. A nickel base alloy of improved characteristics in at least one of stress rupture properties and hot workability, said alloy having a nominal composition consisting essentially of about 0.08% carbon, about 19% chromium, about 9.8% molybdenum, about 11% cobalt, about 3.2% titanium, about 1.5% aluminum, and a balance that is essentially nickel except for an addition in said alloy of yttrium in an amount ranging from about 0.02% to about 0.15%.

\* \* \* \* \*

25

30

35

40

45

50

55

60

65